

## UNITED STATES PATENT OFFICE

2,218,633

## TEXTILE MATERIAL

Angus Smith Bell and Joseph Rowland Wylde,  
Spondon, near Derby, England, assignors to  
Celanese Corporation of America, a corpora-  
tion of Delaware

No Drawing. Application April 5, 1938, Serial No.  
200,145. In Great Britain April 20, 1937

4 Claims. (Cl. 57—140)

This invention relates to improvements in textile materials, and is more particularly concerned with new composite yarns and with fabrics or other materials made of or containing such 5 yarns.

In recent years considerable research has been directed to the production, from artificial textile materials, of yarns which bear a resemblance to natural wool yarns. It has been found that yarns 10 which contain short fibres of artificial textile materials, i. e., artificial staple fibres, are of considerable value in this connection. Such yarns may be made by spinning, in a way comparable to cotton spinning, a roving containing artificial staple fibres, or may be made by processes which comprise treating a bundle of continuous filaments of artificial material so that at least some of such filaments are broken though the continuity of the bundle as a whole is retained. Processes of this latter type are 15 described in U. S. Patents Nos. 2,077,078 and 2,077,079.

It has now been discovered that very valuable composite yarns, having a good resemblance to 5 wool yarns, may be obtained by associating one or more yarns containing artificial staple fibres with one or more yarns which after such association, are capable of being shrunk relative to said yarns containing artificial staple fibres, and 20 thereafter shrinking such shrinkable yarns.

The association of the yarns to form the composite yarns of the present invention may be brought about in any convenient manner. For example the different yarns may be sized together 25 so that they act thereafter as a single yarn until the finished woven fabric or other material is scoured to remove the size. However, it is preferable to bring about the association of the different yarns in the composite 30 yarn by a doubling twist, preferably a light doubling twist.

The staple fibre yarns may have a basis of any artificial material. Thus, they may contain 45 staple fibres having a basis of cellulose acetate or other organic derivatives of cellulose or staple fibres having a basis of regenerated cellulose and produced, for example, by the viscose, cuprammonium or nitrocellulose processes. Or again, the staple fibre yarns may contain staple fibres 50 which have a basis of cellulose acetate or other organic ester of cellulose and which have been partially or completely saponified, or staple fibres which have a basis of an organic derivative of cellulose and which have been subjected to esterification, e. g. by the processes of U. S. applica-

tions S. Nos. 39,289 and 39,290, both filed September 5, 1935.

The staple fibre yarns may be made by any method. Thus they may be made by forming a roving of staple fibres and converting such roving into yarn. Preferably, however, the staple fibre yarns are made by the processes described in U. S. Patents Nos. 2,077,078 and 2,077,079. These processes involve causing a bundle of continuous filaments to pass between two surfaces 10 one of which at least is a cutting surface moving at a speed different from that of the bundle, the other surface serving to press the bundle substantially at a point in its length against the cutting surface. The cutting surface may 15 take the form of a fluted roller as in U. S. Patent No. 2,077,079, or may be an endless cutting band as in U. S. Patent No. 2,077,078, and the pressing surface may be a stationary surface, or may be a surface, for example a roller, moving at substantially the same speed as the cutting roller or surface as in U. S. Patent No. 2,077,078. It is a characteristic of the processes described in these specifications that the conversion of the bundle of continuous filaments 20 into a staple fibre yarn is effected without at any stage losing the continuity of the bundle as a whole. These processes are therefore referred to as "direct conversion" processes.

The shrinkable yarns may be made of any material but it is important that the shrinkable yarn associated with a particular staple fibre yarn should differ in character from the staple fibre yarn so that on treatment with shrinking agents the shrinkable yarn will shrink, whilst 30 the staple fibre yarn remains substantially unaffected or at least shrinks only to a very small extent. This result may be achieved by employing as the shrinkable yarn a yarn which has a basis of a different material from the staple 40 fibre yarn and/or which, by reason of its construction, is especially adapted to be shrunk, e. g. a highly twisted crêpe yarn, (i. e., a yarn twisted to such a degree that it possesses the 45 property of shrinking on treatment with hot aqueous liquors). Thus, for example, there may be associated with staple fibre yarn having a basis of normal cellulose acetate, yarn which has a basis of cellulose acetate of acetyl content higher or lower than normal, e. g. yarn of normal 50 cellulose acetate which has been subjected to acetylation as described, for example, in U. S. applications S. Nos. 39,289 and 39,290, or yarn which has a basis of cellulose acetate which has been ripened to a low acetyl content, e. g., 55

- below 50% acetyl content. Or, again, together with staple fibre yarn having a basis of cellulose acetate or other organic derivative of cellulose there may be employed yarn having a basis 5 of a different derivative of cellulose, of regenerated cellulose, of cellulose acetate or other cellulose ester which has been subjected to partial or complete saponification, or yarns of cotton, silk or wool.
- 10 Where, on the other hand, the staple fibre yarn has a basis of regenerated cellulose, the shrinkable yarn may, for example, have a basis of cellulose acetate or other organic derivative of cellulose or may be a silk or woollen yarn.
- 15 Where the yarn which is associated with the staple fibre yarn is a highly twisted crêpe yarn it is not, in general, necessary that such yarn should be of different material from the staple fibre yarn, since the ordinary aqueous scouring 20 treatments which effect substantial shrinkage of crêpe yarns do not effect any substantial shrinkage of the staple fibre yarns, though where the staple fibre yarns have a basis of cellulose acetate or other organic derivative of cellulose the 25 treatment may crinkle the staple fibres, thus improving their resemblance to natural woollen fibres. The use of crêpe yarns, therefore, presents the advantage that it is possible by means of them to produce composite yarns of uniform 30 chemical character. Another way of obtaining composite yarns which have a uniform chemical character is to employ a staple fibre yarn which is naturally sensitive to shrinking agents and an ordinary yarn of the same character, 35 and to coat the staple fibre yarn with a reserve, e. g., a gum, wax or starch, prior to associating such yarns together, so that on subsequent treatment with a shrinking agent the shrinking agent is prevented by the reserve from acting on the 40 staple fibre yarn. Another process is to associate with a staple fibre yarn containing substantially unstretched artificial fibres a yarn of the same material which has been stretched to a substantial extent. In general stretched yarns 45 are more sensitive to shrinking agents than unstretched yarns so that it is possible by controlling the conditions to effect substantial shrinkage of the stretched yarn without any substantial effect on the staple fibre yarn. Or, again, 50 staple fibre yarn which contains fibres which have been shrunk may be associated with an unshrunk yarn of the same material so that on treatment with a shrinking agent the shrinking effect is restricted almost entirely to the unshrunk yarn.
- 55 It is to be understood, however, that where highly twisted crêpe yarns are employed they are not necessarily made of the same material as the staple fibre yarns. Thus, very satisfactory results may be obtained by associating a cellulose acetate staple fibre yarn with a highly 60 twisted viscose crêpe yarn or a real silk crêpe yarn. Where highly twisted crêpe yarns having a basis of cellulose acetate or other organic derivative of cellulose are employed they are 65 preferably produced by processes in which twist is inserted while the yarn is under the influence of steam or hot water. For such processes reference is made to U. S. Patents Nos. 2,083,628, 2,083,587 and 2,089,191.
- 70 Where the yarn associated with the staple fibre yarn is a highly twisted crêpe yarn the shrinking may be effected, as indicated above, by the ordinary treatments with aqueous scouring liquids. However, in other cases the choice

of shrinking agent will depend on the character of the yarn to be shrunk. For shrinking cotton yarn or yarn having a basis of regenerated cellulose there may be employed, for example, sulphuric or hydrochloric acid, zinc chloride, thiocyanates, e. g. calcium thiocyanate, and other powerful swelling agents for cellulose, whilst for shrinking yarns having a basis of cellulose acetate or other organic derivatives of cellulose agents such as nitric acid or the thiocyanates referred 10 to may be employed. However, these latter yarns are preferably shrunk with the aid of organic shrinking agents, e. g., acetone, and especially methylene chloride or similar latent solvents (see U. S. Patent No. 2,058,422.) 15

As already indicated, the staple fibre yarn and the shrinkable yarn are preferably associated together by a doubling twist. In order to obtain a fabric in which the composite yarn appears to be composed substantially of staple fibre yarn 20 it is preferable that the denier of the staple fibre yarn should exceed substantially the denier of the yarn associated therewith. Thus, for example, a 150-200 denier staple fibre yarn may be very suitably doubled with a 50-100 denier shrinkable yarn. The staple fibre yarn may be permitted to spiral round the shrinkable yarn during the doubling operation, for example by leading the staple fibre yarn to the point where the doubling takes place under a very light tension. 25 Thus, the staple fibre yarn may be fed to the point at which doubling takes place somewhat faster than the shrinkable yarn in order to obtain the desired spiralling effect. The staple fibre 30 yarn may be fed only slightly faster, e. g., 5 or 10% faster, or may be fed considerably faster, e. g., 50-100 or 200% or more faster, according to the nature of the product desired. If this spiralling effect is effected it is not so important that the denier of the staple fibre yarn should 35 substantially exceed the denier of the yarn associated therewith. 40

It will be appreciated that when the yarns are associated by means of a doubling twist the individual component yarns either receive additional twist or have some twist removed therefrom, depending on the relative directions of the doubling twist and the twists in the component 45 yarns. For this reason the twists in the component yarns should be either in excess of, or short of, that desired for them in the composite 50 yarn produced. Thus where it is desired to produce a composite yarn in which the shrinkable component yarn is a high twist crêpe yarn, it is not essential for the yarn fed to the doubling 55 device to be itself a high twist crêpe yarn if, as a result of the addition of the doubling twist, such yarn becomes a high twist crêpe yarn in the product. In using high twist crêpe yarns as the shrinkable yarns it is usually preferable 60 to insert the doubling twist in the same direction as the original twist in such yarns so that at no stage have such yarns a twist higher than that desired for them in the composite yarns. For example, if an ultimate twist of 55 turns 65 per inch in the shrinkable yarn of the composite yarn is desired, it is better to feed the yarns having a twist of 50 turns per inch to the doubling device and increase this to 55 turns per inch by a 5 turns per inch doubling twist in the same 70 direction than to start with a yarn having an original twist of 60 turns per inch and to decrease this to 55 turns per inch by a doubling twist of 5 turns per inch in the reverse direction.

The products produced according to the invention may consist of a single staple fibre yarn doubled with a single shrinkable yarn, e. g., a 170 denier cellulose acetate staple fibre yarn produced by a direct conversion process, doubled with a 75 denier viscose yarn (having, for example, a twist of about 40 turns per inch) with a doubling twist of 5 turns per inch, the doubling twist being in the same direction as the twist in the viscose yarn; or the product may consist of two staple fibre yarns doubled with a single shrinkable yarn, e. g., a composite yarn produced by feeding two 170 denier cellulose acetate staple fibre yarns (produced as indicated above), and a single 75 denier viscose yarn (having a twist of about 33 turns per inch) to a doubling device, the staple fibre yarn being fed 5% faster than the viscose crêpe yarn, and inserting a doubling twist of 12 turns per inch in the same direction as the twist in the viscose yarn.

However, composite yarns produced by doubling together staple fibre yarns and shrinkable yarns may themselves be doubled together to form heavier products and/or or may be doubled with other yarns, e. g., other shrinkable

25 yarns. The composite yarns of the invention may be woven into fabrics in any suitable arrangement. They may, for example, be in the warp or weft 30 or both in the warp and weft, and in any of these cases may be associated with yarns of any other desired character, or composite yarns containing a component having a crêpe twist may alternate in the weft and/or warp with composite 35 yarns containing crêpe components of opposite twist. The invention is of greatest value in connection with the production of woven fabrics but the composite yarns of the present invention may, nevertheless, be formed into fabrics by other fabric-forming operations, for example, by circular knitting or by warp knitting.

40 The treatment of the composite yarns with a shrinking agent may be carried out prior to, or

subsequent to, the conversion of the yarn into fabric form.

The phrase "cellulosic yarns" employed in the claims is to be understood as including yarns having a basis of an organic derivative of cellulose and also yarns having a basis of natural or regenerated cellulose.

Having described our invention, what we desire to secure by Letters Patent is:

1. Process for the production of composite 10 yarns resembling wool yarns, which comprises associating one or more yarns containing artificial staple fibres with one or more yarns which, after such association, are capable of being shrunk relative to such yarns containing artificial staple 15 fibres, and thereafter shrinking said shrinkable yarns.

2. Composite yarns of a wool-like character containing artificial staple fiber yarns doubled with cellulosic yarns, the artificial staple fiber 20 yarns being uniformly cockled by being present in greater length than said cellulosic yarns, and said cellulosic yarns being shrunk to a greater degree than said artificial staple fiber yarns.

3. Composite yarns of a wool-like character 25 containing artificial staple fiber yarns of an organic derivative of cellulose doubled with other cellulosic yarns, the artificial staple fiber yarns being uniformly cockled by being present in greater length than said other cellulosic yarns, 30 and said other cellulosic yarns being shrunk to a greater degree than said artificial staple fiber yarns of an organic derivative of cellulose.

4. Composite yarns of a wool-like character 35 containing artificial staple fibre yarns of cellulose doubled with other cellulosic yarns, the artificial staple fibre yarns being uniformly cockled by being present in greater length than said other cellulosic yarns, and said other cellulosic yarns being shrunk to a greater degree than 40 said artificial staple fibre yarns of cellulose acetate.

ANGUS SMITH BELL.  
JOSEPH ROWLAND WYLDE.

CERTIFICATE OF CORRECTION.

Patent No. 2,218,633.

October 22, 1940.

ANGUS SMITH BELL, ET AL.

It is hereby certified that error appears in the printed specification of the above numbered patent requiring correction as follows: Page 3, second column, strike out lines 10 to 17, comprising claim 1 and for claims now appearing as 2, 3 and 4 read 1, 2 and 3 respectively, and that the said Letters Patent should be read with this correction therein that the same may conform to the record of the case in the Patent Office.

Signed and sealed this 19th day of November, A. D. 1940.

(Seal)

Henry Van Arsdale,  
Acting Commissioner of Patents.